

Patented June 26, 1923.

1,460,048

# UNITED STATES PATENT OFFICE.

PERCY A. E. ARMSTRONG, OF LOUDONVILLE, AND RALPH P. DE VRIES, OF NEWTONVILLE, NEW YORK; SAID DE VRIES ASSIGNOR TO SAID ARMSTRONG.

## ELECTRICAL HEATING ELEMENT.

No Drawing.

Application filed July 29, 1921. Serial No. 488,471.

To all whom it may concern:

Be it known that we, Percy A. E. Armstrong, a subject of the King of Great Britain, and a resident of Loudonville, county of Albany, and State of New York, and Ralph P. De Vries, a citizen of the United States, and a resident of Newtonville, county of Albany, and State of New York, have invented certain new and useful Improvements in Electrical Heating Elements, of which the following is a specification.

Our invention relates to elements for electrical heating purposes, which may be either mechanically worked as by hot or cold rolling, wire drawing or the like, or may be in the form of cast grids or the like. Electrical heating elements in accordance with our invention are made of alloy steel containing iron, chromium, silicon, a high melting point metal or metals other than chromium of the sixth group of Mendel-  
eff's table preferably tungsten, and carbon; and may contain chromium from about 10 to about 30%, silicon from about .5% to 20 about 3.5% or 4% for mechanically worked material, and up to about 6% silicon for cast material, tungsten from about .2% to 25 about 5% for readily mechanically worked material and up to about 10% where the 30 consequent red hardness is not objectionable, carbon from about .05 to about 1%, and the principal part of the remainder is made up of the iron base. The material may contain more or less sulfur or other 35 metalloids, but the proportion of metalloids other than silicon is preferably kept low. Manganese may also be present in the usual proportions encountered in steel making, say up to about 1%. Higher percentages are not desirable, and the manganese may be dispensed with, if desired. Molybdenum or uranium may be substituted for the tungsten or part thereof if desired, with nearly if not quite so good 40 results as with the tungsten.

We have obtained very good results, for example, from electrical heating elements run at about 1700 to 1900° F., and made from alloy steel containing carbon about .20 to .30%, chromium about 17 to 20%, silicon about 2.40 to 3%, tungsten about 2.5 to 3%, manganese about .20 to .40%, and the principal part of the remainder iron, one of several melts being of the following analysis: carbon about .25%, chromium about

18%, silicon about 3%, manganese about .40%, tungsten about 3%, and the principal part of the remainder iron. This material when put into use as an electrical heating element, run up to about the temperatures referred to, shows a smooth whitish surface formation which may be referred to as a frosting or an excessively thin scale, and is subject to practically no progressive deterioration or scale formation in use, so that the body of the metal is not called upon to give up additional metal to form an oxide, and the material stands up extremely well in use over long periods. To obtain this result with a whitish frosting or scale, we have found that at least 2% of silicon should be present and preferably about 2.4%. This whitish frosting appears to some extent with 3% of silicon as used in the foregoing example when as little as .2% of tungsten is used, and with 3% of tungsten as in the foregoing example the whitish frosting effect is obtained to substantially a maximum extent. It appears essential to produce the whitish scale or frosting, which is apparently non-porous and serves as a protection against deterioration of the metal when run at high temperatures, that a considerable body of silicon should be present together with the tungsten. For electrical resistance material used at comparatively low temperature good results can be obtained with silicon as low as about .5%.

The carbon may be as low as about .05% and should not exceed a maximum of about 1%, and preferably should be kept under about .40%. From about .1% or .2% to about .4% of carbon is the best range in order to get best protection against surface deterioration of the metal when run as an electrical heating element, but while carbon above about .4% is not recommended for heating elements, same may be higher up to about 1%, particularly for electrical resistance elements which are used at comparatively low temperatures. The proportions given herein are by weight.

The alloy of the present invention is resistant to rusting and to the action of acids and other corroding agents and may be made use of where these characteristics are of advantage as, for example, it is well adapted for such uses as heating of liquids by means of bare electrical heating ele-

2  
ments submerged in and brought into direct contact with the liquid to be heated.

The specific resistance of elements in accordance with this invention is comparatively high, so that it is possible to make use of elements of relatively small cross-section. For example, elements containing carbon .1 to .4%, silicon 2.4 to 3.5%, tungsten .25 to 5%, manganese under 1%, and the principal part of the remainder iron.

10 the principal part of the remainder—except for chromium—iron, we find that with chromium 17 to 20%, the material has a specific resistance of about 100 microhms per cubic c. c.; with the same material except 15 that the chromium is from 20 to 25%, the specific resistance is about 105 microhms per cubic c. c.; and with 25 to 30% of chromium, the specific resistance is about 110 microhms per cubic c. c.

20 We claim:

1. An electrical heating element made of alloy steel containing carbon about .05 to 1%, chromium more than 10% and less than 30%, silicon about 2 to 6%, a high melting point metal or metals other than chromium of the sixth group of Mendeleff's table about .20 to about 10%, and the principal part of the remainder iron.
2. An electrical heating element made of alloy steel containing carbon about .05 to 1%, chromium more than 10% and less than 30%, silicon about 2 to 6%, tungsten about 20 to 10%, and the principal part of the remainder iron.
3. A mechanically worked electrical heating element made of alloy steel containing carbon about .05 to .4%, chromium about 17 to 25%, silicon about 2 to 3.5%, tungsten about .20 to 5%, and the principal part of the remainder iron.
4. An electrical heating element made of

alloy steel containing carbon about .1 to .4%, chromium about 17 to 25%, silicon about 2.4 to 3.5%, tungsten about 2% to 5%, manganese under 1%, and the principal part of the remainder iron.

5. An electrical heating element made of alloy steel containing carbon about .20 to .30%, chromium about 17 to 20%, silicon about 2.4 to 3%, tungsten about 2.5 to 3%, manganese about .20 to .40%, and the principal part of the remainder iron.

6. An electrical heating element made of alloy steel containing carbon about .1 to .4%, chromium about 18%, silicon about 3%, tungsten about 3%, manganese under 1%, and the principal part of the remainder iron.

7. An electrical heating element made of alloy steel containing carbon, chromium, silicon, tungsten and iron, with at least as much silicon as tungsten and exhibiting a whitish frosting or scale of excessive thinness when subjected to electrical heating at about 1700 to 1900° F.

8. An electrical resistance element made of alloy steel containing carbon about .05 to 1%, chromium about 10 to 30%, tungsten about .20 to 10%, silicon about .5 to 6%, and the principal part of the remainder iron.

9. An electrical resistance element made of alloy steel containing carbon about .05 to 1%, chromium about 17 to 25%, silicon about .5 to 3.5%, tungsten about 2 to 5%, manganese under 1%, and the principal part of the remainder iron.

In testimony that we claim the foregoing, we have signed our names hereto.

PERCY A. E. ARMSTRONG.  
RALPH P. DE VRIES.